

## UNITED STATES PATENT OFFICE

JAMES H. GRAVELL, OF ELKINS PARK, PENNSYLVANIA, ASSIGNOR TO AMERICAN CHEMICAL PAINT COMPANY, OF AMBLER, PENNSYLVANIA, A CORPORATION OF DELAWARE

## FOAM-PRODUCING PROCESS AND MATERIAL FOR ACID METAL-CLEANING BATHS

No Drawing. Application filed March 29, 1927, Serial No. 179,389. Renewed March 20, 1930.

This invention relates broadly to the art of foam production and specifically to the foam produced on acid baths that emit hydrogen.

The objects of the invention are to produce a more permanent foam on acid baths that emit hydrogen; to reduce the cost of foam production; to reduce the heat emanating from the bath; to save acid; to increase the efficiency of the foam and to prevent the escape of acid spray from the bath.

When iron and steel are subjected to the action of an acid bath, such as a dilute solution of sulphuric acid, the acid attacks the metal and liberates hydrogen which bubbles up through the solution and escapes to the air. In so doing, the escaping hydrogen forms unstable bubbles on the surface of the bath, which in breaking, throw an acid mist or spray into the air, to the great detriment of health and materials in the vicinity.

In order to overcome this obnoxious condition, it is the custom to add to the bath a foaming agent, such as saponin, saponin-like materials, rye meal liquor and the like, cellulose pulp waste, etc., which acts to make the bubbles stable, and consequently causes the bath to cover itself with a blanket of foam, which holds the escaping hydrogen long enough to allow its moisture to be precipitated back into the bath eliminating the acid spray.

My experience with the foaming agents indicates that although they are effective, the effect is not permanent, and therefore increments of the foaming agent must be continually added to the bath in order to produce the desired effect. Therefore, in order to maintain a permanent foam, the operator must continually watch the bath and add the agent as conditions require. It should be noted that in the aggregate, so much of the foaming agent is required, that to add the entire amount when the bath is started, would so alter the proportions of the bath that in many cases it would not serve the purpose for which it was intended. The care and attention required to maintain the proper foam on the bath depends so much on human nature that it is often neglected and hence the ob-

noxious fumes often do damage before the oversight is noticed.

I have discovered that by the addition of what I term foam protective materials to the bath in addition to the foaming agent, I can 55 so reduce the amount of foaming agent required that the entire amount of the foaming agent may be added when the bath is made up, without danger of harming the bath, and yet produce a satisfactory foam during the 60 life of the bath.

The best foam protecting material known to me at the present time is formaldehyde, paraformaldehyde, and those materials capable of generating formaldehyde in an acid 65 bath in the presence of metal, such as thioamides and substituted thioamides (all these classes being hereafter included in the term "thioamides"). The thioamides work well with all the foaming agents but from a commercial aspect, I prefer that foaming agent known as cellulose pulp waste liquor.

To practice my invention I may make up an acid bath in a vat using:

|                          | Gallons | 75 |
|--------------------------|---------|----|
| Water                    | 1000    |    |
| Sulphuric acid (66° Bé.) | 50      |    |

Into this bath there may be placed a ton of steel sheets to be cleaned. The bath may be maintained at a temperature of 180° F. 80

To this bath containing the steel, I may add:

|                             |             |    |
|-----------------------------|-------------|----|
| Cellulose pulp waste liquor | .50 gallons | 80 |
| Thiocarbanilide             | 2.00 pounds | 85 |

The bath then begins to develop a foam which collects and forms in a suitable blanket, which materially conserves the heat of the bath and acts as an effective means of separating all moisture from the escaping hydrogen. 90 The blanket thus formed has great lasting powers and without any further additions of the materials referred to above, produces a suitable blanket of foam that endures until the acid is exhausted.

All other conditions being equal, a bath operated without my foam protector would require constant additions of the foaming agent so that in the aggregate it would amount to ten times as much or more.

100

My invention therefore acts to conserve the foaming agent and to materially reduce the attention the bath requires to maintain the blanket of foam.

5 For convenience the foaming agent and the foam protecting material may be compounded in advance and this admixture added to the bath instead of the simple foaming agent. In this case I prefer to use the evaporated cellulose pulp waste liquor which is a solid and I may compound the ingredients as follows:—

|                                        | Pounds |
|----------------------------------------|--------|
| Evaporated cellulose pulp waste liquor | 2.00   |
| Thiocarbanilide                        | 2.00   |

10 15 This results in a powder admixture, in sufficient amount to treat the bath which I have described above.

20 Although I am unable to propose a philosophy to account for the surprising result of materially increasing the longevity of the foam, I am convinced that the presence of the formaldehyde accounts in some unknown manner for it.

25 The following is a definition of thiomide:



30 where  $\text{R}_1$  and  $\text{R}_2$  represent hydrocarbon radicals or hydrogen, and  $\text{R}_3$  represents hydrogen, a hydrocarbon radical, an amino group or a substitute amino group.

It will be obvious to those skilled in the art that the invention is of chemical character, 35 hence I claim the benefit of equivalents appropriate in such cases.

I claim:

40 1. A bath for pickling metal comprising a metal etching acid and water, and further comprising a reaction controlling agent capable of generating formaldehyde in insufficient quantity to stop the generation of hydrogen, and cellulose waste liquor.

45 2. A bath for pickling metal comprising a metal etching acid and water, and further comprising a thioamide body in insufficient quantity to stop the generation of hydrogen, and a foam producing agent.

50 3. A bath for pickling metal comprising a metal etching acid and water, and further comprising thiocarbanilide in insufficient quantity to stop the generation of hydrogen, and a foam producing agent.

JAMES H. GRAVELL.